

Aug. 14, 1928.

1,680,493

S. S. BALL

METHOD OF REMOVING PIPING AND UNSOUND METAL FROM INGOTS

Filed April 24, 1922

FIG. 1.



FIG. 2.



FIG. 3.



FIG. 4.



FIG. 5.



FIG. 6.



FIG. 7.



FIG. 8.



Inventor

Samuel S. Ball,

By Watson, Cott, Morse & Grindle,

Attorneys.

Patented Aug. 14, 1928.

1,680,493

# UNITED STATES PATENT OFFICE.

SAMUEL S. BALL, OF BETHLEHEM, PENNSYLVANIA.

## METHOD OF REMOVING PIPING AND UNSOUND METAL FROM INGOTS.

Application filed April 24, 1922. Serial No. 558,241.

The present invention relates to methods of removing unsound metal from ingots and particularly to methods of removing piping and segregations of impurities from ingot tops.

It has been found, in the manufacture of steel, a practical impossibility to prevent the formation of piping, blow-holes, and segregations of impurities in ingots. The piping occurs centrally of the ingot and at its top for the most part, and is caused by uneven cooling of the metal, as is well known. Segregations of impurities are caused by the forcing of such impurities toward the center of the ingot as the ingot gradually solidifies in cooling from its outer surface toward its center. Generally, the piping and segregation of impurities occur to any considerable extent only at the top of the ingot, the impurities gathering adjacent the bottom of the pipe. To free the ingot of these impurities it has heretofore been generally found necessary to cut off the entire top portion, the volume of which is relatively large as compared with the total volume of the ingot, and to discard this portion.

It has been suggested that the impurities may be removed from ingots and piping prevented, by exerting a pressure thereon while the metal is in a fluid state to force the gases forming in the center of its top and the metal containing impurities gathered at this point, upwardly through a central opening in a descending piston head or die which closely fits within the upper end of the mold in which the liquid metal is contained. In theory the liquid metal which would develop unsoundness if left with the remainder of the metal to solidify is removed by this process, but in practice it is found that a portion only of the impurities is removed, due to the fact that the segregation is not complete when the pressure is applied to the fluid metal, and that piping and segregation still occur within the main body of the ingot and frequently of sufficient seriousness to render the ingot unsuitable for certain purposes.

The present method contemplates the treatment of the ingot while in a plastic state, by means which exerts a pressure on the sound metal surrounding a portion of unsound metal, to force the sound metal toward the body of the ingot to displace the unsound metal. This unsound metal is forced outwardly and forms a projection

which may be easily removed. The method may be employed to remove unsound metal from any part of an ingot providing it is adjacent the outer surface where it may be observed, but is principally employed in the removal of the unsound metal and piping from the top of the ingot.

Pressure is applied only after the piping has been completely formed and the segregation of impurities completed. An ingot in a plastic state, which may have been heated as a preparatory step, or which may be cooling after having been cast, is disposed vertically in a confining die which is slightly larger in horizontal cross section than the ingot. Pressure is then exerted by an upsetting die upon the upper surface of the ingot to flatten out this upper surface and to shorten and thicken the ingot so that it bears against the wall of the confining die at all points. A displacement die is then applied to the top of the ingot, which has a central recess in its bottom of considerable size leaving a narrow marginal surface around this recess which is adapted to bear on the sound metal at the sides of the ingot. Downward movement of the displacement die causes the sound metal of the margins of the ingot to be forced into the body of the ingot to displace the unsound metal, this metal flowing upwardly and entering the recess in the displacement die. When the operation has been completed the unsound metal is nearly all contained in the knob or lug projecting from the upper end of the ingot and when this is removed the ingot is practically free of localized segregations of impurities.

In addition to effecting the isolation of the impurities in this manner so that they may be removed with a minimum of loss of metal, there are a number of other advantages flowing from the application of the method. The action of the upsetting and displacement dies on the metal results in the refining of its structure and particularly the refinement of the surface metal. Blow-holes throughout the ingot are closed up. The base knobs or projections which protrude from the bottom of the ingot due to erosion of the mold stool, are eliminated. In addition, only a short time is required to carry out the method, several minutes only being necessary, whereas when an ingot in the fluid stage is treated an hour or more is necessary. Furthermore, the displacement

of the metal in accordance with the present method may be carried out to any desired extent, it being within the power of the operator to stop the movement of the die at any point.

Where the ingot is to be subjected to a subsequent rolling operation, as in the case of the fabrication of rails, I beams, or other structural shapes, the method is particularly beneficial. The compression of the ingot longitudinally and expansion laterally while in the confining mold is exactly the reverse of the process of rolling, in which the ingot is reduced in section and increased in length. The working of the metal as a preliminary step in a manner exactly the reverse of that in which it is worked in a subsequent rolling operation, improves the physical qualities of the steel and refines the grain so that the resulting rolled articles are of superior quality.

In the accompanying drawings:

Figure 1 is a central longitudinal section through a typical ingot as it comes from a casting mold;

Figure 2 shows the ingot in section, the bottom of the ingot resting in a cup die which forms part of the confining die;

Figure 3 shows the ingot completely enclosed by the confining die and with the up-setting die in operative position;

Figure 4 shows the condition of the ingot at the completion of the movement of the up-setting die;

Figure 5 shows the displacement die in operative position;

Figure 6 shows the displacement die at the completion of its movement;

Figure 7 illustrates the ingot in vertical section at the completion of the last step and after removal from the confining die; and

Figure 8 is a section on the line 8—8 of Figure 6.

The ingot illustrated in Figure 1 is typical of those produced in large quantities in the manufacture of steel and has a body portion 10, an axial depression 11 or pipe in its upper surface, and irregular knobs 12 projecting from its lower end due to the wearing away or erosion of the mold in which it was cast. Around the base of the pipe 11 is a portion 13 of metal which is unsound due to the inclusion of impurities or segregations. It is sought to remove the pipe 11 and the unsound metal 13, and the first step of the process is to place the ingot, which is in a heated and plastic state, on a plate 14 with the lower end of the ingot resting in a cup-shaped depression 15 formed in the plate. The two halves 16 of a separable die are then brought together to enclose the ingot, the portions 16 forming, with the plate 14, a confining die completely surrounding the ingot except at the top. The inner walls of the die are spaced somewhat from the

outer wall of the ingot, as shown in Figure 3, the space within the walls of the confining die being greater in cross section than the ingot. The up-setting die 17 is next applied to exert a downward axial pressure on the ingot which shortens and thickens it and causes it to expand laterally to fit against the walls of the die, as shown in Figure 4.

The up-setting die is now removed and replaced by the displacement die 18. This displacement die has a central stepped recess 19 in its lower end, the margins only of the lower face of the die being adapted to bear initially on the ingot. Both the up-setting and displacement dies are provided with small central conduits 20 so that air and gas may escape during the compression operations. Downward movement of the displacement die results in the compression of the sound metal around the edges of the top of the ingot and the forcing of this metal downwardly into the main body of the ingot. As a result of this movement the central portion of the ingot top is displaced and moves upwardly and if the die 18 is moved downwardly sufficiently, the recess 19 may be completely filled with metal, as shown in Figure 6.

When the operation has been completed the ingot is removed from the confining die and it will then be seen that the piping has been eliminated and that the unsound metal has been isolated and is all within the lug or projection extending axially from the ingot top. This projection may be severed without difficulty, leaving the remainder of the ingot free from unsoundness. The bottom of the ingot has also been rounded and the lugs 12 removed. Not only is the piping removed and impurities of the ingot isolated in a minimum of time, but the grain structure of the metal is refined during the operation and its physical properties improved. The method is especially useful where the ingot is to be subsequently rolled, the steps of the above described method when combined with the steps of a rolling operation, resulting in a structural shape of high quality. While the method is described as applied to an ingot of well known type having a square cross section, it will be understood that it is equally applicable to round ingots or ingots of any shape.

Having thus described my invention what I claim as new and desire to secure by Letters Patent is:

1. The method of freeing the body of an ingot of piping and segregations in the top thereof which includes the step of applying forces to the ingot entirely in a direction truly axial of the latter and when the latter is in a plastic state to effect the flattening of the upper end of the ingot, and the step of applying forces entirely in an axial di-

rection to the margins of the ingot top to force the sound marginal metal into the body of the ingot and to displace the centrally located unsound metal.

- 5 2. The method of treating ingots having unsound terminal core portions surrounded by sound metal which consists in applying forces to the end of the ingot having the unsound terminal core portion and axially 10 of the ingot to secure contraction of the unsound core portion and thickening of the sound metal surrounding the latter and then in applying forces axially of the compressed ingot and in annular zones to the sound 15 metal surrounding the contracted core portion to secure further compression of the ingot and the extrusion of the unsound metal of the core portion.
3. The method of forming rolled articles 20 consisting in pouring an ingot, cooling the ingot below the temperature at which blow holes and segregates are completely formed,

heating the ingot to a temperature at which it becomes plastic, applying pressure to the sound metal surrounding the metal containing the blow holes and segregates to extrude the latter beyond the main portion of the ingot, and then rolling the ingot.

4. The method of forming rolled articles consisting in pouring an ingot, cooling the 30 ingot below the temperature at which the blow holes and segregates are completely formed, heating the ingot to a temperature at which it becomes plastic, compressing the ingot through its entire length, applying 35 pressure to the sound metal surrounding the metal containing the blow holes and segregates to extrude the latter beyond the main portion of the ingot, and then rolling the 40 ingot.

In testimony whereof I hereunto affix my signature.

SAMUEL S. BALL.